

## UNITED STATES PATENT OFFICE

2,197,380

## ELECTRIC CONTACT ELEMENT

Franz R. Hensel and Kenneth L. Emmert,  
Indianapolis, Ind., assignors to P. R. Mallory &  
Co., Inc., Indianapolis, Ind., a corporation of  
Delaware

No Drawing. Application June 2, 1939,  
Serial No. 277,016

2 Claims. (Cl. 200—166)

This invention relates to improvements in electric contact elements.

It is an object of the invention to provide a contact which possesses superior physical properties such as high specific gravity and satisfactory strength.

It is a further object of the invention to provide a contact of high melting point and high recrystallization temperature.

10 Other objects of the invention will be apparent from the following description, taken in connection with the appended claims.

The present invention comprises a combination of elements, methods of manufacture and the 15 product thereof, brought out and exemplified in the disclosure hereinafter set forth, the scope of the invention being indicated in the appended claims.

While a preferred embodiment of the invention 20 is described herein, it is contemplated that considerable variation may be made in the method of procedure and the combination of elements without departing from the spirit of the invention.

25 According to the present invention, an improved contact is contemplated, formed of an alloy having the following ingredients present in substantially the ranges of proportion given below:

|                                                   |          |
|---------------------------------------------------|----------|
| 30                                                | Per cent |
| Uranium                                           | .1 to 35 |
| Refractory metal of the tungsten-molybdenum group | Balance  |

35 Part of the refractory metal can be replaced by rhenium. We have found that it is possible to produce tungsten base materials containing up to 35% of uranium, part of which is taken up by tungsten in solid solution and part of which 40 exists as a free constituent, the bonded alloys showing increased hardness and considerable resistance to abrasion. Uranium is suitable as an alloy element for tungsten because it has a melting point of 1700 to 1800 degrees C. Uranium and tungsten can be sintered by heating to a 45 temperature above 1200 degrees C. in a non-oxidizing atmosphere, such as in vacuum.

We have also found that such elements as carbon, boron, or silicon, may be added. Our 50 experiments have shown that uranium will form compounds with these elements and when added to our improved tungsten-uranium alloys double compounds may be formed. We have found that alloys of the following composition show 55 considerable advantages—

|             | Per cent |
|-------------|----------|
| A. Tungsten | 99.50    |
| Uranium     | .50      |
| B. Tungsten | 95.00    |
| Uranium     | 5.00     |
| C. Tungsten | 75       |
| Molybdenum  | 10       |
| Rhenium     | 10       |
| Uranium     | 5        |
| D. Tungsten | 65       |
| Uranium     | 35       |
| E. Tungsten | 75       |
| Uranium     | 25       |
| F. Tungsten | 35       |
| Molybdenum  | 35       |
| Uranium     | 30       |

In our experiments we have found that alloys with low uranium contents can be manufactured 20 by mixing the powders, subjecting same to a high pressure to form an ingot. The ingot or special shapes then may be sintered and forged or swaged, rolled or drawn to a convenient shape from which the various parts can be manufactured, 25 for which this alloy is particularly suitable. Binary alloys of high uranium content are difficult to swage and must be manufactured by a sintering process only.

This swaging difficulty, however, can, in certain cases, be overcome if other elements of the tungsten group are added, such as molybdenum or rhenium. Tests conducted on the use of the alloys described for electrical make and break contacts indicated that the material has good 35 properties both as far as contact resistance and material transfer are concerned. This is the case, both if the materials are operated against each other or against a contact of this composition or under polarized conditions.

We have found that the desirable characteristics described above will not be disturbed if small proportions of other ingredients are present from the iron group materials, such as iron, cobalt and nickel, or small percentages of tantalum, columbium, chromium and manganese.

We have also found that we can use our new alloying composition as a refractory base for a material composition consisting of high melting point materials taken from the group molybdenum, tungsten, rhenium and containing substantial quantities of uranium impregnated with low melting point materials taken from the group copper, silver, gold, platinum and palladium and their alloys.

Since certain changes in producing the above alloy and certain modifications in the composition which embody the invention may be made, without departing from its scope, it is intended that all matter contained in the above description shall be interpreted as illustrative and not in a limited sense.

It is also to be understood that the following claims are intended to cover all of the generic and specific features of the invention herein described and all statements of the scope of the

invention, which as a matter of language might be said to fall therebetween.

What is claimed is:

1. An electric contact element formed of an alloy of .1 to 35% uranium and the balance substantially all tungsten.

2. An electric contact element formed of a metal composition containing at least 65% tungsten and .1 to 35% uranium.

FRANZ R. HENSEL.  
KENNETH L. EMMERT.

10